

## UNITED STATES PATENT OFFICE

2,436,138

## PHOTOGRAPHIC EMULSIONS OF SILVER SALTS IN HYDROPHILIC POLYMERS OF 1,3-DIOXOLANE

Theodore Le Sueur Cairns, Roselle, and David Malcolm McQueen, Newark, Del., assignors to E. I. du Pont de Nemours & Company, Wilmington, Del., a corporation of Delaware

No Drawing. Application November 27, 1944,  
Serial No. 565,402

4 Claims. (Cl. 95—7)

1

This invention relates to photographic emulsions and emulsion layers composed of hydrophilic polymers of 1,3-dioxolane and to photographic elements containing the same.

In the past many different materials have been used in photographic emulsions as binding agents for the light-sensitive components. The most widely used binder, gelatin, is well adapted to this use because it serves as a good protective colloid for silver halides in fluid emulsions and when coated on a suitable support and dried, these emulsions form films which are permeable to the aqueous solutions used to develop the photographic images. However, gelatin has some disadvantages among which may be mentioned its high cost, which is due largely to the time-consuming preparatory processes necessary to give a product of high purity. Further, gelatin is not uniform in quality and varies from one lot to another. Other disadvantages of gelatin include its susceptibility to bacterial attack and the deleterious effect of changing humidity. That is, at high relative humidity gelatin films become soft and weak unless given a special hardening treatment and under conditions of low relative humidity they are very brittle.

Other materials have been tried as binding agents but have met with little success. For example, collodion, one of the first binders used for silver halides, is very insensitive to water and must be processed in special fashion. Albumin, agar-agar, casein, and other natural colloids have also been tried as emulsion binders but all have many disadvantages such as high cost, low film strength, too high or too low water sensitivity, etc. More recently, it has been proposed to use certain derivatives of polyvinyl alcohol and cellulose derivatives. However, gelatin remains the best binder now available and it is used in almost all light-sensitive emulsions that are commercially available.

An object of this invention is to provide new photographic emulsions and emulsion layers which are free from the disadvantages of gelatin. Another object is to provide such emulsions which can be prepared in a simple and economical manner. Another object is to provide new photographic emulsions from synthetic materials which are of uniform quality. A still further object is to provide novel photographic emulsions which are not susceptible to bacterial attack. Still other objects are to reduce the cost of photographic emulsions and improve their resistance to changes of humidity.

It has been found that useful photographic 55

2

compositions can be made by incorporating radiation-sensitive materials in a hydrophilic polymer of 1,3-dioxolane. This may be accomplished by colloidally dissolving the polymer of 1,3-dioxolane in water and admixing the light-sensitive material therewith. After the light-sensitive material has been uniformly dispersed, the resulting solution may be further modified and coated onto a support to form a light-sensitive layer.

- 10 In a preferred mode of the invention, the hydrophilic polymer of 1,3-dioxolane is dissolved in an aqueous solution and light-sensitive silver halides are precipitated therein. This may advantageously be accomplished by dissolving a soluble ionizable halide, e. g., sodium, potassium or ammonium chloride or bromide, etc., in the solution of the polymer of 1,3-dioxolane and adding an aqueous solution of a soluble ionizable silver salt, e. g., silver nitrate, with stirring. The resulting emulsion can then be ripened, chilled or precipitated, digested and modified by the addition of more of the same 1,3-dioxolane polymer, general emulsion sensitizers, anti-fogging agents, spectral sensitizing dyes, preservatives, hardeners and/or color formers, etc., and coated onto a temporary or permanent support or onto a layer of such support. Unwashed emulsions can be used but in general it is desirable to remove the excess soluble salts. For example, the unwashed emulsion may be precipitated with a salt solution such as an aqueous sodium sulfate solution, washed free from soluble salts and then redissolved in a fresh 1,3-dioxolane polymer solution.

After the light-sensitive 1,3-dioxolane polymer solution is prepared for coating it may be deposited, in the same way that gelatin silver halide solutions are coated, upon a suitable support, e. g., metal, paper, glass, or a transparent film such as cellulose nitrate, cellulose acetate, nylon, etc., and dried. The resulting element can then be exposed and processed to positive or negative pictures in the same manner as ordinary gelatin silver halide photographic elements.

The hydrophilic polymers of 1,3-dioxolane 45 which have been found to be useful in the photographic emulsions and layers described above can be made after the manner described in Gresham application Serial No. 392,124, filed May 6, 1941, now United States Patent 2,394,910, by polymerizing 1,3-dioxolane at a temperature between  $-80^{\circ}$  C. and  $300^{\circ}$  C. and preferably between  $0^{\circ}$  C. and  $150^{\circ}$  C. at normal, sub- or super-atmospheric pressure. Generally, excellent results are obtained at atmospheric pressure but pressures from 1 to 100 atmospheres may be used.

If desired, the temperature of the reaction, especially when polymerization is carried out at the boiling point of the cyclic compound, may be controlled by varying the pressure on the boiling reactants.

It has been found advantageous to effect the polymerization in the presence of a catalyst such, for example, as sulfuric acid, phosphoric acid, hydrochloric acid, hydrofluoric acid (alone or with  $\text{BF}_3$ ), boron fluoride (including its complexes with water, acids, esters, alcohols, and the like), para-toluenesulfonic acid, camphor sulfonic acid and other acid catalysts of this general nature. Friedel-Crafts type catalysts other than  $\text{BF}_3$  may be used such as  $\text{AlCl}_3$ ,  $\text{AlBr}_3$ ,  $\text{FeCl}_3$ , etc., as may be inorganic acids generally, and their acid salts such as sodium acid sulfate, sodium acid phosphate, etc.

The reaction is carried out for an extended period until solid polymers which are capable of cold drawing are formed. This reaction is preferably carried out at moderate temperatures, e. g., 20° to 80° C. at about normal pressure, for a period of several days using boron trifluoride as a catalyst.

It is believed that the polymerization proceeds in accordance with the equation



wherein  $x$  is at least 135. The polymers comprehended by the present invention in terms of molecular weight have a weight of at least 10,000. The useful polymers can best be selected by their viscosity characteristics. They should have a relative viscosity of at least 1.04 (determined as 0.1% in chloroform) and from 1.06 to 1.20 represents a practical range. By relative viscosity is meant the viscosity in comparison to that of pure chloroform to which is assigned a value of 1.00. All viscosities are at 25° C.

The 1,3-dioxolane polymers used in accordance with this invention are generally soluble in water at 40° to 60° C. to the extent of 5-20% or more but, if desired, water containing small amounts (10-20%) of a water-soluble organic solvent, e. g., ethanol, methanol or another monohydric alcohol of less than 4 carbon atoms, may be employed. Aqueous solutions of the hydrophilic polymers of 1,3-dioxolane are stable at ordinary temperatures but when heated to 80° C. to 100° C. precipitation of the polymers occurs. This unusual property may be used advantageously in manufacturing the polymers for this invention.

The invention will be further illustrated by the following examples. All parts are by weight.

#### Example I

A reaction mixture containing 400 parts of 1,3-dioxolane and about 0.2 part of boron trifluoride is allowed to stand at room temperature for 5 days. At the end of this time, the polymer, which is a hard, tough, resin-like solid, is converted to thin shavings which are dissolved in 0.1% aqueous  $\text{NH}_4\text{OH}$  at 50° to 60° C. and precipitated from this solution at 100° C. after adding 3-4 parts of  $\text{NaOH}$  for every 50 parts of polymer dissolved. The catalyst-free polymer is then spread on a smooth surface such as a glass or metal plate and allowed to dry for 5 to 50 hours. If desired, the drying process may be accelerated by placing the polymer in a vacuum oven and drying at 50° C. The dry polymer is cut into small pieces and pressed into a thin film by heating on the platens

of a press at 100° C. under a pressure of approximately 100 lbs./sq. in. for 5-30 minutes. The properties of this treated film are:

- 5 Appearance \_\_\_\_\_ Tough, elastic, white.  
 Tensile strength \_\_\_\_\_ 3020 lbs./sq. in.  
 Elongation at break \_\_\_\_\_ 425%.  
 Elongation recovery \_\_\_\_\_ 325%.  
 Film appearance \_\_\_\_\_ Colorless, cloudy, flexible.  
 10 Cold draws well and stretches in the cold drawn state.  
 Molecular weight \_\_\_\_\_ 86,000 (determined by viscosity of a chloroform solution).  
 15 Melting point \_\_\_\_\_ 63°-70° C.

#### Example II

A mixture is made of 15 parts of 3 N ammonium bromide, 2 parts of 0.5 N potassium iodide and 20 5.0 parts of a 10% solution of the hydrophilic polymer of 1,3-dioxolane (prepared according to Example I) and, while stirring at 40° C., a solution of 10 parts of 3 N solution of silver nitrate containing sufficient ammonium hydroxide to 25 give a clear solution is added slowly. The photographic emulsion thus formed is stirred at 40° C. for 15-60 minutes, cooled, and coated on a support. After drying, the photographic element is exposed to an object and developed by immersion 30 at 18°-30° C. in a standard p-methylaminophenol-hydroquinone developer such as the following:

|                              | Parts |
|------------------------------|-------|
| p-Methylaminophenol sulfate  | 3     |
| Sodium sulfite (anhydrous)   | 45    |
| 35 Hydroquinone              | 12    |
| Sodium carbonate (anhydrous) | 67.5  |
| Potassium bromide            | 1.9   |
| Water to make                | 1000  |

40 The developed picture is fixed by bathing in a 25% solution of sodium thiosulfate (hypo), freed of soluble salts by washing, and dried. The resulting black and white picture has density gradations complementary to the object scene to which 45 the element was exposed.

#### Example III

A photographic silver halide emulsion prepared as in Example II is precipitated by adding an 50 excess of saturated solution of sodium sulfate and then washed free of soluble salts in running water. The emulsion is then redissolved in 50 parts of 10% polymer solution and digested at 50°-60° C. for 30-60 minutes. The washed emulsion thus 55 obtained is coated and processed as in Example II to obtain a black and white negative picture.

#### Example IV

A gelatin-silver halide photographic emulsion 60 (100 parts) is warmed to 35° C. and diluted with 100 parts of water and centrifuged. The silver halide precipitate thus obtained is washed free of gelatin by centrifuging and redispersed in 100 parts of 10% solution of polydioxolane containing 65 1 part of a 5% solution of sodium dodecylsulfate by stirring rapidly at 30° C. for 15-30 minutes. The resulting light-sensitive emulsion is coated and processed as in Example I to obtain a black and white negative picture of good quality.

#### Example V

A reaction mixture containing 400 parts of 1,3-dioxolane and about 0.2 part of boron trifluoride was allowed to stand for 13 days at 6° C. In three days the mixture became viscous and in 7 days

had solidified. Thin shavings of the resultant solid polymer were dissolved in approximately 0.1% aqueous NH<sub>4</sub>OH at 50°-60° C. and precipitated from this solution at 100° C. after adding 3-4 parts of sodium hydroxide for every 50 g. of polymer dissolved. The catalyst-free polymer is then spread on a smooth surface such as a glass or metal plate and allowed to dry for 5 to 50 hours. If desired, the drying process may be accelerated by placing the polymer in a vacuum oven and drying at 50° C. The dry polymer is cut into small pieces and pressed into a thin film by heating on the platens of a press at 100° C. under a pressure of approximately 100 lbs./sq. in. for 5-30 minutes. The properties of this treated film are:

|                        |                                                                                                                      |
|------------------------|----------------------------------------------------------------------------------------------------------------------|
| Appearance             | Tough, elastic, white.                                                                                               |
| Tensile strength       | 4520 lbs./sq. in.                                                                                                    |
| Elongation at break    | 600%                                                                                                                 |
| Elongation recovery to | 250%                                                                                                                 |
| Film appearance        | Colorless, translucent, non-tacky, flexible, tough. Cold draws well and has considerable stretch in cold drawn state |
| Molecular weight       | 196,000 (determined by viscosity method in chloroform)                                                               |

Cold drawn film:

|                        |                   |
|------------------------|-------------------|
| Tensile strength       | 5530 lbs./sq. in. |
| Elongation at break    | 200%              |
| Elongation recovery to | 50%               |

Example VI

A mixture is made of 15 parts of 3 N ammonium bromide, 2 parts of 0.5 N potassium iodide and 5.0 parts of a 10% solution of the hydrophilic polymer of 1,3-dioxolane (prepared according to Example V) and, while stirring at 40° C., a solution of 10 parts of 3 N solution of silver nitrate containing sufficient ammonium hydroxide to give a clear solution is added slowly. The photographic emulsion thus formed is stirred at 40° C. for 15-60 minutes, cooled, and coated on a support. After drying, the photographic element is exposed to an object and developed by immersion at 18°-30° C. in a standard p-methylaminophenol-hydroquinone developer such as the following:

|                              | Parts |
|------------------------------|-------|
| p-Methylaminophenol sulfate  | 3     |
| Sodium sulfite (anhydrous)   | 45    |
| Hydroquinone                 | 12    |
| Sodium carbonate (anhydrous) | 67.5  |
| Potassium bromide            | 1.9   |
| Water to make                | 1000  |

The developed picture is fixed by bathing in a 25% solution of sodium thiosulfate (hypo), freed of soluble salts by washing, and dried. The resulting black and white picture has density gradations complementary to the object scene to which the element was exposed. In preparing polymers of 1,3-dioxolane, monofunctional compounds can be added to the polymerization reaction mixture in small amounts in order to react with the polymer units at the end of the polymeric chain provided, however, that the amount of monofunctional compound added does not reduce the molecular weight of the polymer below 10,000. Such monofunctional compounds include carboxylic acids and their acid chlorides and anhydrides, sulfonic acids, sulfonyl halides, and the

like. Suitable specific compounds include acetyl chloride, propionyl chloride, butyryl chloride, valeryl chloride, benzoyl chloride, and toluoyl chloride and the corresponding acids and anhydrides, ethane sulfonyl chloride, cyclohexanesulfonyl chloride, benzene sulfonyl chloride, para-toluenesulfonic acid, etc. When used in small amounts as chain terminating agents, these compounds do not modify to any material extent the properties of the poly-1,3-dioxolane as a gelatin substitute.

The invention, moreover, is not limited to the specific light-sensitive material described in the above-detailed examples. On the contrary, various other simple and mixed silver halides may be used as the light-sensitive materials in like manner.

15 Mixtures of silver bromides, chlorides and/or iodides can be made by adding mixtures of soluble salts of these halides in like manner.

20 Other useful soluble halides include potassium bromide, potassium iodide, sodium and potassium chlorides and iodides, etc. Other useful soluble silver salts include silver sulfamate, silver sulfate, silver citrate and silver acetate.

25 Still other radiation-sensitive or light-sensitive materials such as light-sensitive diazonium compounds, ammonium bichromate, fulgides, etc. can be used in the emulsions and emulsion layers composed of the above hydrophilic 1,3-dioxolane polymers.

30 The emulsions, after formation, are preferably digested at a temperature from 40° to 80° C. for a period of from 30 minutes to 6 hours. During the digestion stage or prior thereto, various types

35 of sensitizing agents, e. g., sulfur sensitizers such as allylthioureas, thiocyanates, sodium thiosulfate, allylthiocyanates, can be added. In addition, various types of optical sensitizing dyes which modify the spectral characteristics of the

40 resulting emulsions can be added. Suitable sensitizing dyes are described in U. S. Patents 2,010,388, 2,079,376, 2,202,990, 2,202,991, 2,202,992, 2,278,461, 2,265,908, etc.

45 Various types of color formers or dye intermediates capable of forming quinoneimine or azomethine dyes on color-forming development can be incorporated in the emulsions. Thus, the phenols, naphthols, pyrazolones, acylacetamides, hydridene, N-homophthalylamines, etc., particularly those of high molecular weight and which are immobile in gelatin emulsion layers can be used. Suitable color formers are described in

50 U. S. Patents 2,108,602, 2,166,181, 2,178,612, 2,179,228, 2,179,238, 2,179,239, 2,182,815, 2,184,303, 55 2,186,849, 2,200,924, 2,283,276, and 2,328,652.

55 The hydrophilic 1,3-dioxolane polymer emulsions are normally used without other film-forming colloids. However, they are compatible to a limited extent with gelatin and certain other materials, such as cellulose derivatives, and these may be added to the light-sensitive compositions if desired.

60 The photographic elements of the present invention have a number of outstanding advantages over the prior art materials. For example, they are based on a material derived from formaldehyde and ethylene glycol and thus offer substantial economic advantages. The photographic emulsions have great stability toward bacterial and fungal decomposition and this is also true of the coated photographic elements. This inertness is perhaps related to the chemical structure of the 1,3-dioxolane polymer which derives its hydrophilic character from the plurality of in-

trilinear ether groups in contrast to other materials proposed as photographic colloids.

Surprisingly, the hydrophilic 1,3-dioxolane polymers are also soluble in certain hydrocarbon solvents and, for example, can be removed from the support by treatment with benzene. This is an advantage in simplifying scrap film recovery. The film elements also are free from the brittleness characteristics of gelatin films.

The light-sensitive film elements of the present invention may be used, for example, as a taking stock (negative), as print stock (positive), or as reversal film, in the preparation of films for microcopy, V-mail, in X-ray films, in lithographic films and in portrait materials. In addition, when diazonium salts or ammonium bichromate are incorporated in hydrophilic polymers of 1,3-dioxolane to form the light-sensitive layers, the film elements may be used in the graphic arts and in the reproduction of line drawings. In fact, the film elements of this invention can be used in any way in which elements based on gelatin or collodion have been used.

What is claimed is:

1. A photographic element comprising a support bearing at least one layer composed of a hydrophilic polymer of 1,3-dioxolane which polymer contains a large number of recurring units of the formula  $-\text{CH}_2\text{OCH}_2-\text{CH}_2-\text{O}-$ , has a molecular weight of at least 10,000 and a relative viscosity of 1.06 to 1.20 when present in an amount of 0.1% by weight in chloroform, said layer containing a light-sensitive silver salt.

2. A photographic element comprising a support bearing at least one layer composed of a hydrophilic polymer of 1,3-dioxolane which polymer contains a large number of recurring units of the formula  $-\text{CH}_2\text{OCH}_2-\text{CH}_2-\text{O}-$ , has a molecular weight of at least 10,000 and a relative viscosity of 1.06 to 1.20 when present in an amount of 0.1% by weight in chloroform said layer having uni-

formly dispersed therethrough light-sensitive silver halides.

3. A photographic element comprising a support bearing at least one layer composed of a hydrophilic polymer of 1,3-dioxolane said layer containing a color former and light-sensitive silver salts, said polymer having a large number of recurring units of the formula



10 a molecular weight of at least 10,000 and a relative viscosity of 1.06 to 1.20 in chloroform when present in a concentration of 0.1% by weight.

15 4. A photographic emulsion composed of a hydrophilic polymer of 1,3-dioxolane which polymer contains a large number of recurring units of the formula  $-\text{CH}_2\text{OCH}_2-\text{CH}_2-\text{O}-$ , has a molecular weight of at least 10,000 and a relative viscosity of 1.06 to 1.20 when present in an amount of 0.1% by weight in chloroform said layer having dispersed therethrough a light-sensitive silver halide.

THEODORE LE SUEUR CAIRNS.  
DAVID MALCOLM McQUEEN.

#### 25 REFERENCES CITED

The following references are of record in the file of this patent:

#### 30 UNITED STATES PATENTS

| Number       | Name           | Date          |
|--------------|----------------|---------------|
| 2,187,081    | Hodgins et al. | Jan. 16, 1940 |
| 2,276,322    | Lowe           | Mar. 17, 1942 |
| 2,350,350    | Gresham        | June 6, 1944  |
| 35 2,360,477 | Dahle          | Oct. 17, 1944 |
| 2,366,737    | Loder et al.   | Jan. 9, 1945  |
| 2,394,910    | Gresham        | May 6, 1941   |

#### 35 FOREIGN PATENTS

| Number  | Country       | Date          |
|---------|---------------|---------------|
| 496,049 | Great Britain | Nov. 21, 1938 |